

[54] ALUMINIUM BASED ALLOY WITH A HIGH YOUNG'S MODULUS AND HIGH MECHANICAL, STRENGTH

[75] Inventor: Jean-Francois Faure, Voiron, France

[73] Assignee: Pechiney Recherche, Courbevoie, France

[21] Appl. No.: 503,903

[22] Filed: Apr. 4, 1990

[30] Foreign Application Priority Data

Apr. 5, 1989 [FR] France ..... 89 04700

[51] Int. Cl.<sup>5</sup> ..... C22C 21/10

[52] U.S. Cl. ..... 148/11.5 A; 148/12.7 A;  
420/532; 428/659

[58] Field of Search ..... 148/11.5 A, 12.7 A;  
420/532; 428/659

[56] References Cited

U.S. PATENT DOCUMENTS

- 3,563,814 2/1971 Lyle et al. ..... 148/12.7  
3,791,876 2/1974 Kroger ..... 148/2  
4,462,843 7/1984 Baba et al. ..... 148/11.5 A  
4,711,762 12/1987 Vernam et al. ..... 148/11.5 A  
4,747,890 5/1988 Meyer ..... 420/532  
4,830,826 5/1989 Ichiro ..... 420/532  
4,874,578 10/1989 Homberger et al. ..... 148/11.5 A

FOREIGN PATENT DOCUMENTS

- 0081441 6/1983 European Pat. Off. ....  
0105595 4/1984 European Pat. Off. ....  
0213850 12/1983 Japan ..... 148/11.5 A

Primary Examiner—Roy Upendra  
Attorney, Agent, or Firm—Dennison, Meserole, Pollack & Scheiner

[57] ABSTRACT

The invention concerns aluminum based alloys of the 7000 series with a high Young's modulus ( $E \geq 74$  GPa), high mechanical strength ( $R_{0.2} \geq 530$  MPa in the longitudinal direction), good tenacity (KIC, longitudinal direction  $\geq 20$  MPa $\sqrt{m}$ ), and good resistance to corrosion under tension ( $\sigma \geq 250$  MPa in the short transverse direction, durability  $\geq 30$  days ASTM standard G 38-73. The alloy according to the invention is of the following composition by weight: from 5.5 to 8.45% of Zr; from 2 to 3.5% Mg; from 0.5 to 2.5% up to 0.5% Fe; up to 0.5% Si; other elements  $\leq 0.05\%$  each; and up to 0.15% in all with  $0.1 \leq Zr \leq 0.5$   $0.3 \leq Cr \leq 0.6\%$ ; and  $0.3 \leq Mn \leq 1.1\%$ . It is preferably worked by the following process steps: a solid body of the composition claimed above is formed by spray deposition; the body is converted to a worked product, at from 300° to 450° C., the optionally converted cold; and the worked product undergoes heat treatment comprising dissolution, quenching and annealing in a T6 or T7 state.

3 Claims, 1 Drawing Sheet





FIG. 1



FIG. 2



FIG. 3

## ALUMINIUM BASED ALLOY WITH A HIGH YOUNG'S MODULUS AND HIGH MECHANICAL STRENGTH

### BACKGROUND OF THE INVENTION

#### 1. Field of the Invention

The invention concerns aluminium based alloys of the 7000 series, in the nomenclature of the Aluminium Association (AA), with a high Young's modulus and good mechanical properties of resistance and tenacity; it also concerns a method of obtaining them.

#### 2. Description of the Related Art

Aluminium alloys of the 7000 series, among the most resistant, generally have a Young's modulus E of the order of 70 GPa but not more than 72-73 GPa.

However, the need for light alloys with a higher Young's modulus ( $F \geq 74$  GPa) and high resistance ( $R_{0.2} \geq 530$  MPa in the longitudinal direction) is felt in order to lighten structures, particularly in the aeronautical and space fields. These properties must be obtained without markedly prejudicing other use properties such as tenacity (KIC, longitudinal direction  $\geq 20$  MPa  $\sqrt{m}$ ) or resistance to corrosion under tension (non-rupture threshold after 30 days  $\geq 250$  MPa in the short transverse direction and in the test medium in question).

Aluminium based alloys containing Li with a high modulus of elasticity and good mechanical properties are indeed known. However, their working poses complex problems given the reactivity of the Li, and special, expensive working and casting installations are required. The alloys according to the invention can be worked in conventional installations such as are known in the metallurgy of common Al alloys. Moreover the mechanical resistance properties of Al-Li alloys are generally inferior to those of 7000 alloys.

Type 7000 alloys, which are much more charged with alloy elements and obtained by metallurgical treatment of powders, have good mechanical properties and good resistance to corrosion under tension, but a modulus of less than 74 GPa.

### SUMMARY OF THE INVENTION

The invention thus concerns alloys of the following composition by weight (%)

|                |                   |
|----------------|-------------------|
| Zn:            | 5.5-8.45          |
| Mg:            | 2.0-3.5           |
| Cu:            | 0.5-2.5           |
| Zr:            | 0.1-0.5           |
| Cr:            | 0.3-0.8           |
| Mn:            | 0.3-1.1           |
| Fe:            | up to 0.5         |
| Si:            | up to 0.5         |
| other elements | each $\leq 0.05$  |
| Remainder Al   | total $\leq 0.15$ |

The following is a preferred composition:

|     |         |
|-----|---------|
| Zn: | 7.0-8.4 |
| Mg: | 2.0-2.9 |
| Cu: | 0.8-2.0 |
| Zr: | 0.1-0.4 |
| Cr: | 0.3-0.6 |
| Mn: | 0.3-0.9 |

the remainder being identical with the above compositions.

A method of obtaining the alloys comprises:

1. forming a solid body of a composition within the above limits, by spray deposition.

2. converting the body hot into a worked product at from 300°-450° C. then possibly converting it cold.

3. applying heat treatment by dissolving the alloy, quench hardening and annealing it, in a T6 or preferably T7 state as defined by the AA.

### BRIEF DESCRIPTION OF THE DRAWING

FIGS. 1-3 are graphs of mechanical properties versus  $R_{0.2}$  for alloys according to and outside the range of the invention.

### DETAILED DESCRIPTION OF THE INVENTION

Spray deposition is understood as being a process in which the metal is melted and sprayed by a jet of high pressure gas in the form of fine liquid droplets, which are then directed onto and agglomerated on a substrate to form a solid cohesive deposit containing slight closed porosity. The deposit may be in the form of billets, tubes or plates of controlled geometry. A method of this type is known as "spray deposition" in the Anglo Saxon world and is also described as the "OSPREY" process. The latter process is chiefly described in the following patent applications (or patents): GB-B-1379261; GB-B-1472939; GB-B-1548616; GB-B-1599392; GB-A-2172827; EP-A-225080; EP-A-225732; WO-A-87-03012.

The hot conversion stage may be preceded by treatment to homogenise the solid body. This may take place in one or more stages at temperatures from 450° to 520° C. and generally lasting 2 to 50 hours.

The product thus obtained has the required properties mentioned above. These properties are attributed to fine dispersion of type (Al, Mn, Cr) phases and  $Al_3Zr$ —due to the combination of the composition of the alloy and the method by which it is obtained. With this structure it is possible to obtain inter alia good ductility, tenacity and a high elastic limit.

Dissolution is generally effected at from 450°-520° C. and the type T6 treatment at from 90° to 150° C., for long enough substantially to obtain peak hardness (2 to 25 hours).

The T7 treatment comprises a type T6 treatment plus annealing at a high temperature, e.g. from 150° to 170° C., for 0.5 to 20 hours.

The invention may also be applied to composite materials hardened by dispersed ceramic particles of the oxide, carbide, nitride, silicide, boride type etc. These are included in the alloy according to the invention, which forms the matrix for them during operation 1, e.g. with powder being injected into the liquid flux.

The particles are from 1 to 50 microns in size and represent a fraction by volume (relative to the metal) of from 3 to 12%.

The invention will be understood better from the description of the following tests: alloys numbers 1 to 4 are according to the invention, alloys 5 and 6 beyond the scope of the invention and alloy 7 is a conventional prior art one (7075) which is given for comparison; it has been cast semi-continuously, converted hot and subjected to the same heat treatment as the other alloys. FIG. 1 shows the mechanical properties E and  $R_{0.2}$  of the alloys tested, FIG. 2 the tenacity properties as a

function of  $R_{0.2}$  and FIG. 3 the corrosion under tension properties as a function of  $R_{0.2}$ .

### EXAMPLE

Various alloys, numbered 1 to 6 and of the percentage weight compositions given in Table 1, are melted and worked by spray deposition (OSPREY process) in billet form.

casting temperature: 750° C.

distance from spray to deposit: 600 mm, kept substan-

lus and elastic limit are low, so it cannot be distinguished from conventional alloys such as 7075.

The composition and properties of a conventional alloy 7075 are given as a comparison. This alloy has been cast in the conventional manner then converted and given the same range of heat treatments as alloys 1 to 6.

The modulus and elastic limit of this alloy will be seen to be well below those for the alloys according to the invention.

TABLE 1

| Alloy             | Zn  | Mg  | Composition alloys tested |      |      |      |       |       |           |
|-------------------|-----|-----|---------------------------|------|------|------|-------|-------|-----------|
|                   |     |     | Cu                        | Cr   | Mn   | Zr   | Fe    | Si    | Remainder |
| 1                 | 7.8 | 2.3 | 1.4                       | 0.35 | 0.85 | 0.16 | <0.1  | <0.1  | Al        |
| 2                 | 8.0 | 2.4 | 1.35                      | 0.45 | 0.50 | 0.17 | <0.1  | <0.1  | Al        |
| 3                 | 6.5 | 2.2 | 1.5                       | 0.50 | 0.60 | 0.20 | <0.1  | <0.1  | Al        |
| 4                 | 7.0 | 2.3 | 1.4                       | 0.35 | 0.40 | 0.18 | <0.1  | <0.1  | Al        |
| 5                 | 7.5 | 2.2 | 1.35                      | 0.9  | 1.2  | 0.25 | <0.1  | <0.1  | Al        |
| 6                 | 6.0 | 2.2 | 1.5                       | 0.15 | 0.18 | 0.12 | <0.1  | <0.1  | Al        |
| 7075 conventional | 5.5 | 2.3 | 1.6                       | 0.23 | —    | —    | <0.05 | <0.04 | Al        |

TABLE 2

Properties of alloys tested (state T7)

| Alloy             | Traction lengthwise |             |      | Traction in long transverse direction |             |      | Modulus (GPa) | Tenacity* L-T direction (MPA $\sqrt{m}$ ) | Corrosion** in tension (nonrupture 30 days) (MPa) |
|-------------------|---------------------|-------------|------|---------------------------------------|-------------|------|---------------|-------------------------------------------|---------------------------------------------------|
|                   | $R_{0.2}$ (MPa)     | $R_m$ (MPa) | A %  | $R_{0.2}$ (MPa)                       | $R_m$ (MPa) | A %  |               |                                           |                                                   |
| 1                 | 580                 | 620         | 9.0  | 550                                   | 590         | 7.0  | 76            | 22.5                                      | 310                                               |
| 2                 | 590                 | 630         | 8.5  | 560                                   | 595         | 6.5  | 75.5          | 21.8                                      | 310                                               |
| 3                 | 535                 | 600         | 12.0 | 520                                   | 570         | 9.2  | 76.4          | 30.8                                      | 310                                               |
| 4                 | 575                 | 610         | 10.0 | 550                                   | 580         | 8.5  | 74.5          | 35.2                                      | 280                                               |
| 5                 | 582                 | 612         | 3.0  | 540                                   | 555         | 1.5  | 78.2          | 12.0                                      | 240                                               |
| 6                 | 520                 | 550         | 13.1 | 500                                   | 525         | 8.2  | 72.5          | 35.9                                      | 310                                               |
| 7075 conventional | 470                 | 536         | 14.5 | 428                                   | 501         | 14.2 | 72.0          | 45.0                                      | 310                                               |

\*Longitudinal stress, spreading crack in transverse direction

\*\*Tests in short transverse direction in accordance with ASTM G 38 73.

tially constant during test

stainless steel collector with rotating movement spray oscillated relative to axis of rotation of collector gas delivery/metal delivery 2 to 3  $m^3/kg$ .

After being scalped to 140 mm diameter, the billets are homogenised for 8 hours at 460° C. The blanks are then hot drawn at 400° C. in a press where the container member has a diameter of 143 mm, in the form of flat parts 50×22 mm in section, giving a drawing ratio of 14.6. The flat parts thus obtained undergo type T7 heat treatment under the following conditions:

dissolving for 2 hours at from 460° to 485° C.

quenching with cold water

two stage annealing: 24 hours at 120° C. + one 20 hour stage from 155° to 170° C.

The mechanical properties obtained are given in Table 2.

Alloys 1 to 4 are within the scope claimed. They have a modulus  $\geq 74$  GPa, an elastic limit in the longitudinal direction  $\geq 530$  MPa, with good ductility in the longitudinal direction ( $\geq 8\%$ ) and the long transverse direction ( $\geq 6\%$ ), tenacity in the L-T direction of at least 20 MPa  $\sqrt{m}$  and good resistance to corrosion under tension (measured in accordance with ASTM standard G 38 73).

Alloy 5 is outside the scope of the invention because its Cr and Mn content is too high, and although it has a high modulus and a high elastic limit it is very inflexible and cannot be used for manufacturing parts. Alloy 6 is also outside the scope of the invention, because its Cr and Mn content is too low. It does not have the advantages of the alloys according to the invention; its modu-

40 The alloys according to the invention are chiefly designed for the manufacture of sections or pieces of forged or swaged structures.

I claim:

1. A spray deposited, hot worked, aluminum-based alloy, consisting essentially of, by weight:

5.5-8.45% Zn;

2-3.5% Mg;

0.5-2.5% Cu;

0.1-0.5% Zr;

0.3-0.6% Cr;

0.3-1.1% Mn;

up to 0.5% Fe;

up to 0.5% Si;

other elements  $<0.05\%$  each, up to 0.15% total; and remainder Al,

55 said alloy having the mechanical properties:

$E \geq 74$  GPa

$R_{0.2}$  (longitudinal dir.)  $\geq 530$  MPa

KIC (longitudinal dir.)  $\geq 20$  MPa  $\sqrt{m}$

Resistance to corrosion under tension (30 days, short transverse dir.)  $\geq 250$  MPa.

2. A spray deposited, hot worked, aluminum-based alloy, consisting essentially of, by weight:

7.0-8.4% Zn;

2-2.9% Mg;

0.8-2.0% Cu;

0.1-0.4% Zr;

0.3-0.6% Cr;

0.3-0.9% Mn;

up to 0.5% Fe;  
 up to 0.5% Si;  
 other elements <0.05% each, up to 0.15% total; and  
 remainder Al,  
 said alloy having the mechanical properties:  
 $E \geq 74 \text{ GPa}$   
 $R_{0.2} \text{ (longitudinal dir.)} \geq 530 \text{ MPa}$

KIC (longitudinal dir.)  $\geq 20 \text{ MPa} \sqrt{\text{m}}$   
 Resistance to corrosion under tension (30 days, short  
 transverse dir.)  $\geq 250 \text{ MPa}$ .  
 3. An alloy according to claim 1 or 2, containing a  
 5 homogeneous dispersion of ceramic particles from 1 to  
 15 microns in size and representing a fraction by vol-  
 ume, (relative to the metal) of from 3 to 12%.

\* \* \* \* \*

10

15

20

25

30

35

40

45

50

55

60

65